

July 18, 1972

P. VOHL

3,677,717

APPARATUS AND METHOD FOR PRODUCING II-VI CRYSTALS

Filed March 6, 1969



PAUL VOHL  
INVENTOR.

BY *David E. Brook*

ATTORNEY.

## 1

3,677,717

### APPARATUS AND METHOD FOR PRODUCING II-VI CRYSTALS

Paul Vohl, Lexington, Mass., assignor to Itek  
Corporation, Lexington, Mass.  
Filed Mar. 6, 1969, Ser. No. 804,895  
Int. Cl. B01j 17/30

U.S. Cl. 23—294

13 Claims

#### ABSTRACT OF THE DISCLOSURE

Apparatus is disclosed for nucleating and growing II-VI crystals such as zinc selenide. The apparatus comprises a hollow reaction vessel having walls constructed of an inert, high-temperature resistant material and having an outlet passageway with a much smaller cross-sectional area than that of the reaction vessel, the reduction in area occurring immediately adjacent to the point of crystal nucleation. This apparatus also contains a means for heating the reaction vessel to temperatures of at least about 400° C.

A process for nucleating and growing II-VI crystals using a throttling technique is also disclosed.

The apparatus and process disclosed are useful for producing single, pure, defect-free II-VI crystals which are in turn useful in electro-optic applications.

#### BACKGROUND OF THE INVENTION

##### (I) Field of the invention

This invention relates to an apparatus and process for producing II-VI crystals and more particularly relates to an apparatus and process for producing single, pure, defect-free II-VI crystals by a vapor transport technique.

##### (II) Description of the prior art

Nucleation and growth of II-VI crystals has heretofore been accomplished by the use of temperature gradients. For example, Piper and Polich have disclosed an apparatus wherein a sealed crucible containing a II-VI source material and a nucleation point is moved through a temperature gradient. See "Vapor-Phase Growth of Single Crystals of II-VI Compounds," Journal of Applied Physics, vol. 32, No. 7, July 1961, pp. 1278-9. Nucleation and growth with this apparatus and technique is directly proportional to the rate at which the crucible is moved through the temperature gradient.

De Meis and Fischer have taught an apparatus for preparing II-VI crystals which consists of a quartz ampoule having a sealed capillary tube attached to one end of the ampoule. See "Improved Method for Growing II-VI Crystals From the Vapor Phase," Materials Research Bulletin, vol. 2, 1967, pp. 465-8. The purpose of the capillary in this apparatus is to adjust the minimum vapor pressure within the system by collecting excess volatile material until the decomposition pressure in the ampoule has reached its minimum. In use, the ampoule is evacuated to a pressure of  $10^{-6}$  Torr, sealed, and moved through a temperature gradient furnace. Crystal growth initiates in the hotter portion of the capillary tube thereby sealing it off.

Frosch, U.S. 3,197,411, issued July 27, 1965, teaches an apparatus for growing single crystals of the III-V semiconductor compounds, gallium phosphide and gallium arsenide, on suitable substrates. This apparatus consists of a fused silica tube which has gas inlets and which extends through two temperature controlled furnaces designed to produce a temperature gradient within the apparatus. The source is contained in a quartz boat at a high temperature end. The substrate material is positioned further down the quartz tube at a lower temperature. A

## 2

small gas outlet is positioned well beyond the substrate where the crystal nucleates and grows. Nucleation and growth of the III-V crystals is caused by the temperature gradient maintained between the source and growth surface (see col. 2, lines 31-33). Since the apparatus operates on a thermal gradient principle, it can function equally well as both an open system and closed system (see col. 2, lines 28-31).

All of the above-described apparatus and processes depend on saturated vapor in a temperature gradient for crystal nucleation and growth. None suggest that crystallization from the vapor phase can be accomplished by other techniques.

#### SUMMARY OF THE INVENTION

It has now been found that nucleation and growth of single II-VI crystals from a carrier gas saturated with vaporized source material can be accomplished by simply throttling the carrier and vapor species. This is completely unexpected.

Relying on this finding, a novel and unique apparatus for nucleating and growing crystals containing at least one Group II-B element and at least one Group VI-A element selected from sulphur, selenium, and tellurium has been invented.

This apparatus comprises a hollow reaction vessel having walls constructed from an inert, high-temperature resistant material such as quartz. A carrier gas is admitted to the reaction vessel through glass tubing or by other means and is exited from the reaction vessel through a passageway having a much smaller cross-sectional area ( $A_2$ ) than that of the reaction vessel ( $A_1$ ). The reduction in areas creates a substantial throttling effect on the carrier gas and other vapor species which in turn causes crystal nucleation and growth to commence. Heating means are used to vaporize the source material.

A process for nucleating and growing II-VI crystals from a source material containing a Group II-B element or a Group VI-A element selected from sulphur, selenium, and tellurium has also been invented. This process takes advantage of the throttling phenomenon.

In the process, the source is contacted with a flow of carrier gas and heated to a temperature sufficient to saturate the vapor phase with the elements to be crystallized. The saturated vapor phase is then throttled to cause crystal nucleation and growth.

The apparatus and process of this invention offer many advantages over what has been heretofore known in the prior art. For example, higher growth rates with concomitant shortened running times can be obtained with the claimed apparatus and process. Another important advantage is that crystal grows "free"—i.e. mechanically unconstrained by chamber walls or crucibles and such free growth results in improved crystal properties. Furthermore, the apparatus is simple in construction and operation and therefore offers a more economical means of growing crystals. Another advantage is that the apparatus can be maintained at atmospheric pressure thereby eliminating complicated and expensive equipment to maintain low vacuums or superatmospheric pressures. A further advantage of this apparatus and process is that the single crystals of II-VI materials produced are unusually pure and defect-free. Also very large crystals can be grown. Additionally, the apparatus and process herein disclosed make seeding unnecessary to obtain crystal nucleation. Also, the system automatically insures that stoichiometric conditions are maintained because excess volatile materials are exhausted. Exhausting the excess volatile materials also results in higher purity crystals. While the excess volatile materials are exhausted, it has been found that very little of the vaporized source material escapes from the apparatus of this invention. This is because the vaporized source material is

cooled in the exit means and therefore condenses before it can escape to the open atmosphere.

A further advantage to the apparatus and process of this invention is that they provide a means to achieve the nucleation and growth of a single crystal nucleus at a desired, predetermined point location. Furthermore, they prevent extraneous nucleation at other undesirable points.

#### BRIEF DESCRIPTION OF THE FIGURE

The figure is a partially cut away schematic diagram of apparatus for nucleating and growing II-VI crystals according to this invention.

#### DESCRIPTION OF THE INVENTION

This invention is related to an apparatus and a process for growing crystals of II-VI elements. For purposes of this invention, the elements referred to as II or Group II elements are more specifically those elements of Group II-B—i.e., zinc, cadmium and mercury. In a like manner, the VI or Group VI elements useful with this invention are more specifically Group VI-A elements selected from sulfur, selenium and tellurium. The terms "II," "VI," "Group II-B" and "Group VI-A" refer to groupings found in a periodic chart of the elements such as the one found opposite page 1 of The Condensed Chemical Dictionary, 7th ed. For brevity, the crystals produced will often be referred to as "II-VI" crystals.

The apparatus claimed contains a hollow reaction vessel having walls constructed from an inert high temperature resistant material such as glass, quartz, or a ceramic material such as mullite. This vessel has a cross-sectional area  $A_1$ . Of course, the vessel does not have to have a circular cross-sectional area, although this is one preferred embodiment, Square, triangular, elliptical, etc. cross-section areas would also be suitable for the reaction vessel, as would any other shape including irregular shapes.

A means for admitting a carrier gas is connected to the front portion of the apparatus. Any suitable means such as glass, plastic, or rubber tubing are suitable to allow entrance of the carrier gas. A particularly preferred means for admitting the carrier gas is a capillary tube integrally attached to the front of the reaction vessel because such a capillary helps to prevent back diffusion of the carrier gas and vaporized material due to temperature gradients within the reaction vessel.

An exit passageway is provided to allow the carrier gas to leave the reaction vessel. This exit passageway has a cross-sectional area  $A_2$  which is sufficiently smaller than  $A_1$  to create a throttling effect on the carrier gas and vaporized source material as they pass from the reaction vessel into the exit passageway. It is this throttling effect that causes nucleation to commence. The theory of why such a throttling effect causes nucleation is not presently known, but it has been repeatedly observed that nucleation commences immediately adjacent to the point of such throttling. Because of this, it is important to position the reduction of cross-sectional areas from the reaction vessel to the exit means immediately adjacent to the point at which it is desired to nucleate and grow the crystal.

The cross-sectional areas of the reaction vessel and exit means do not have to be uniform. Where they are not however, the areas  $A_1$  and  $A_2$  are the areas immediately prior to and immediately past the location where the reaction vessel and exit means are joined. The reduction in areas from  $A_1$  to  $A_2$  has to be substantial to attain crystal nucleation and growth. It has been found that a ratio of  $A_2/A_1$  should normally be in the range of from about 1/40 to about 1/10,000, and preferably is in the range of from about 1/3,000 to about 1/5,000 for the best results.

The apparatus also has a means of heating the reaction vessel to temperatures of at least about 400° C. and to much higher temperatures if they are required to vaporize specific source materials. The heating means can be any well-known type of heater such as a resistance heater, inductance heater, etc. A particularly preferred

heating means is one which can provide a temperature gradient within the reaction vessel. The higher temperature is maintained at the source and the lower temperature is maintained at the nucleation and growth end of the reaction vessel. Although a temperature gradient is not required, it has been found to result in faster crystal growth rates, especially after the initial nucleation and growth period.

The proper temperatures for the source and point of crystallization will depend, of course, upon many factors including the particular Group II-B and Group VI-A elements to be crystallized. In general, the source will have to be heated to and maintained at a temperature sufficient to achieve a vapor phase saturated with a Group II-B element and a Group VI-A element and the point of crystallization can be maintained at about the same temperature or preferably at a somewhat lower temperature. As one illustration of this, it has been found desirable to maintain a zinc selenide source in the range of from about 1150° C. to about 1230° C. while maintaining the point of crystallization at a temperature of about 0-50° C. lower.

One embodiment of the apparatus for producing single II-VI crystals is shown in the figure. The reaction vessel 1 comprises a cylindrical piece of quartz tubing with a capillary tube 2 integrally attached to it to allow the gas to enter the reaction vessel and a capillary tube 3 also integrally attached to it to allow the carrier gas to pass from the reaction vessel. The source material 4 is positioned at the front end of the apparatus and can be contained or uncontaminated. A heater 5 is positioned about the reaction vessel. As the carrier gas enters the reaction vessel 1 through the capillary tube 2, and passes the heated source 4, it transports vaporized source material from the heated source material 4. The carrier gas transports the vaporized source material through the reaction vessel to the joining point for the capillary tube 3 and reaction vessel 1, where the carrier gas and vaporized source material are throttled causing nucleation to commence at point 7. The single crystal 8 grows inwardly towards the center of the reaction vessel 1 unconstrained by the vessel walls. An inlet tube 9 and an outlet tube 10 can be respectively positioned before the capillary tube 2 and after the capillary tube 3. Such inlet and outlet tubes simply serve to admit and exhaust the carrier gas.

It has been found that apparatus as described above with entrance and exit capillaries having inside diameters of about 0.25 to about 3 millimeters and with a reaction vessel having an inside diameter of about 5 to about 100 millimeters, all being circular in cross-section, produce excellent results.

A process for nucleating and growing II-VI crystals from a source material as described above will now be described.

Initially, the source material is heated to a temperature sufficient to saturate the vapor phase while the source is contacted with a flow of an inert carrier gas. The vaporized source material is transported by the carrier gas, and nucleation and crystal growth are initiated by throttling the flow of carrier and vaporized source material.

For this process, the source must contain either a Group II-B element or one of the Group VI-A elements. It may contain more than one element of each group. If it only contains one of the Group II-B or Group VI-A elements, the other required element to produce the II-VI crystals can be introduced as part of the carrier gas. In the preferred embodiment of this invention, a Group II-B and a Group VI-A element are included in the source material.

As stated above, the source material is heated to an elevated temperature. The exact temperature will vary with the particular source material, but will be known or easily ascertainable by those skilled in the art.

The carrier gas flow is introduced so that it comes into intimate contact with the heated source material. Since

the source material has been heated to an elevated temperature the vapor species become saturated with vaporized source material.

Many gases are sufficient as carriers including hydrogen, nitrogen, argon, and helium. Others will be apparent to those skilled in the art.

The carrier gas can contain a Group II-B element or a Group VI-A element which is to form part of the crystal being grown. Hydrogen sulfide ( $H_2S$ ) and hydrogen selenide ( $H_2Se$ ) are examples of such gases. Additionally, doping gases or gases containing a constituent useful in forming mixed crystals can be used as carrier gases.

The saturated vapor phase is transported by the carrier gas from the source to a crystallization point. As explained above, the temperature at the point of crystallization does not have to differ from that at the source to obtain nucleation. Preferably, however, the temperature at the point of crystallization is somewhat lower than that at the source because such a temperature gradient results in faster crystal growth.

At the point where crystallization is desired, the carrier gas and saturated vapor phase are throttled sufficiently to cause nucleation. This can be accomplished by any suitable means, as for example, by forcing the gas and source vapor through an orifice or capillary tube. Nucleation commences immediately adjacent to the point at which throttling occurs.

Although the process and apparatus of applicant have heretofore been described in terms of producing II-VI crystals containing at least one Group II-B element and one Group VI-A element, it will be clear to those skilled in the art that mixed crystals can also be produced. Some examples of such mixed crystals include those having the following formulas:

$BeS_xSe_{(1-x)}$ ,  $Be_xZn_{(1-x)}S$ ,  $ZnSe_xTe_{(1-x)}$ ,  $Zn_xCd_{(1-x)}Se$ , 35  
 $CdSe_xTe_{(1-x)}$ ,  $Cd_xHg_{(1-x)}Te$ ,  
 $HgSe_xTe_{(1-x)}$ ,  $Zn_yCd_{(1-y)}Se_xTe_{(1-x)}$  and  
 $CdS_x(Se_xTe_{(1-x)})_{(1-x)}$

where  $x$  and  $y$  each have a numerical value greater than 40 zero and less than one.

It will also be clear to those skilled in the art that the II-VI crystals can be doped with various other elements. This can be accomplished by a variety of techniques which would include, for example, placing a doping material inside the reaction vessel close to or with the source material or by introducing a doping material combined with the carrier gas. Some examples of well-known doping agents include in particular the elements of boron, 45 aluminum, gallium, indium, phosphorus, arsenic, antimony, and copper as well as many others known to those skilled in the art.

The apparatus and process described herein are both useful in producing single, pure II-VI crystals of exceptionally large size. These crystals are in turn useful in electro-optic applications such as image-converters, image storage and retrieval systems, and light-emitting devices.

The following example illustrates the invention. All parts and percentages are by weight unless otherwise specified.

#### EXAMPLE

The reaction vessel is a quartz ampoule cylindrical in shape and having a uniform inside diameter of about 30 millimeters along its length of about 9 centimeters. Capillary tubes 0.5 millimeter in diameter and about 3 centimeters in length are integrally attached at both ends. The reaction ampoule also has a side arm attachment for the purpose of loading the source material. Six millimeter diameter quartz end tubes are attached to the capillary tubes leading from the reaction ampoule. The reaction vessel is surrounded with a wire wound resistance heated furnace about 14 inches in length with a core opening of 2 inches. The furnace is suitably insulated with fire brick. The quartz end tube protrudes out of the furnace to pro-

vide a room temperature condensation zone for residual vapors.

Approximately 40 grams of powdered or sintered zinc selenide is loaded into the reaction ampoule through the side arm. The side arm is then sealed off near the ampoule and removed. All traces of source powder are carefully removed from the deposition zone by torching while a reverse flow of argon drives the vapor to the front end of the reaction chamber. The ampoule is then installed into the furnace and hydrogen gas lines are attached to the end tubes. The furnace is raised to a temperature of about 1220° C. Hydrogen flow is maintained at about 3 cubic centimeters per minute.

Nucleation is observed to have occurred at the entrance to the exit capillary tube after two days. The crystal continues to grow towards the center of the reaction ampoule. While some crystallites do condense in the capillary tube, at no time during the run is the capillary tube clogged. Vapor flow is continuous throughout the run. As the crystal grows into the space of the reaction ampoule, the throttling effect diminishes and growth can be accelerated by cooling the growth area to a temperature of 0 to 50° lower than the temperature at the source material. The run is continued under these conditions for a total of 8 days at which time a single, pure defect-free zinc selenide crystal of 20 grams is produced.

What is claimed is:

1. Apparatus for using a vapor transport technique to nucleate and grow crystals of at least one Group II-B element and at least one Group VI-A element selected from sulfur, selenium, and tellurium, said apparatus comprising:

- (a) a hollow reaction vessel having walls constructed from an inert, high-temperature resistant material, said reaction vessel having a cross-sectional area  $A_1$ ;
- (b) means for admitting a carrier gas to said reaction vessel;
- (c) an exit passageway having a single flow area with an effective diameter of from about 0.25 millimeter to about 3 millimeters and having a cross-sectional area  $A_2$  which is sufficiently smaller than  $A_1$  to create a substantial throttling effect on the carrier gas and vaporized source material, the ratio  $A_2/A_1$  being in the range of from about  $\frac{1}{3000}$  to about  $\frac{1}{5000}$ , the reduction from  $A_1$  to  $A_2$  being located immediately adjacent to the point at which crystal nucleation and growth is desired;

- (d) means for heating said reaction vessel to temperatures of at least about 400° C., said means for heating being capable of producing a temperature gradient within the reaction vessel, the temperature at the source being higher than the temperature at the point of crystal nucleation and growth.

2. Apparatus of claim 1 wherein said means for admitting a carrier gas is a capillary tube having an inside diameter of from about 0.25 millimeter to about 3 millimeters.

3. Apparatus of claim 2 wherein said reaction vessel has an inside diameter at  $A_1$  of from about 5 millimeters to about 100 millimeters.

4. Apparatus of claim 3 wherein said means for heating the reaction vessel comprises a resistance heater.

5. A process for nucleating and growing II-VI crystals from a vapor phase saturated with at least one Group II-B element and at least one Group VI-A element selected from sulfur, selenium and tellurium, comprising:

- (a) contacting a source of said Group II-B and said Group VI-A elements with a flow of carrier gas;
- (b) heating said source to a temperature sufficient to achieve a vapor phase saturated with said Group II-B and said VI-A elements;
- (c) reducing the flow area at the point of condensation by providing a single flow area at said point having an effective diameter of from about 0.25 millimeter to about 3 millimeters to throttle the flow of said

saturated vapor phase and to limit nucleation thereby effecting single crystal growth.

6. A process of claim 5 wherein the temperature at the source is maintained higher than the temperature at the point of crystal nucleation and growth.

7. A process of claim 6 wherein said source material contains zinc selenide.

8. A process of claim 6 wherein said source material contains zinc sulfide.

9. A process of claim 6 wherein said source material 10 contains zinc telluride.

10. A process of claim 7 wherein said carrier gas is selected from the group consisting of hydrogen, nitrogen, helium and argon.

11. A process of claim 7 wherein said carrier gas comprises hydrogen.

12. A process of claim 11 wherein said source is maintained at a temperature in the range of from about 1150° C. to about 1230° C.

13. A process of claim 12 wherein said point of crystal nucleation and growth is maintained at a temperature of

from 0° C. to about 50° C. lower than the temperature maintained at the source material.

References Cited

5

UNITED STATES PATENTS

|           |         |                |        |
|-----------|---------|----------------|--------|
| 3,031,261 | 4/1962  | Vogel et al.   | 23—294 |
| 3,058,812 | 10/1962 | Li Chu et al.  | 23—273 |
| 3,104,365 | 9/1963  | Broser et al.  | 23—294 |
| 3,199,961 | 8/1965  | MacAvoy et al. | 23—294 |
| 3,218,204 | 11/1965 | Ruehrwein      | 23—294 |
| 3,224,912 | 12/1965 | Ruehrwein      | 23—294 |
| 3,338,761 | 8/1967  | Cheney et al.  | 23—273 |
| 3,353,914 | 11/1967 | Pickar         | 23—301 |
| 3,362,795 | 1/1968  | Weisbeck       | 23—301 |
| 3,525,594 | 8/1970  | Barrett        | 23—273 |

NORMAN YUDKOFF, Primary Examiner

R. T. FOSTER, Assistant Examiner

20

U.S. CL. X.R.

23—273, 301, 305